

Feb. 10, 1931.

A. W. BURWELL

1,791,860

PAPER SIZING AGENT

Filed Dec. 11, 1926



## UNITED STATES PATENT OFFICE

ARTHUR W. BURWELL, OF NIAGARA FALLS, NEW YORK, ASSIGNOR TO ALOX CHEMICAL CORPORATION, OF NEW YORK, N. Y., A CORPORATION OF NEW YORK

## PAPER-SIZING AGENT

Application filed December 11, 1926. Serial No. 154,201.

This invention relates to products particularly adapted for use as paper sizing agents, to the process of making the same, and to papers sized with these products.

5 Papers commonly are sized by one of two methods; "engine-sizing", wherein the sizing agent is added to the pulp in the beating engine and subsequently precipitated on the fibers in an insoluble condition, and "tub-sizing", wherein the sizing operation is carried out on the paper-machine. The product of the present invention is more particularly adapted for use in the "engine-sizing" operation.

15 Heretofore, the only agent widely used in the "engine-sizing" operation has been rosin or colophony, which is said to consist principally of an acid body,—abietic acid. An aqueous solution of the sodium salt of this body, obtained by dissolving rosin in a solution of an alkali, customarily is added to paper pulp in the beating engine and the soluble sodium salt converted to the insoluble aluminum salt of said acid body by treatment with

25 a soluble aluminum salt.

The above described rosin size, although very widely used, is known to lack certain desirable characteristics and to possess certain undesirable characteristics. For example, 30 rosin size possesses imperfect water-repelling properties. Also, there is encountered great difficulty in retaining it in the paper stock in an amount greater than about 8% of the finished, sized paper, due to the fact that the 35 insoluble rosin salt cannot be sufficiently fixed or mordanted on the cellulose fibers. This undesirable characteristic may partially account for the fact that only very limited quantities of inert materials (i. e., fillers) can be 40 incorporated in the paper pulp, since it is believed that the fillers are retained therein only by virtue of the sizing agent.

One object of the present invention is to 45 provide a sizing agent which shall possess the desirable characteristics of rosin size while avoiding the disadvantages above referred to. Among the advantageous characteristics to be desired are a more pronounced water-repelling property, a more nearly perfect mordanting ability, and an ability to retain relatively

larger amounts of inert materials (fillers) in the paper stock.

I have found that, by the liquid-phase oxidation, under controlled conditions, of hydrocarbons or mixtures thereof such as those occurring in petroleum oils, there may be obtained organic acid products, and that these may serve as starting materials for the production of valuable new paper sizing agents. By suitably controlling the conditions, it is possible to produce such agents possessing characteristics that are varied within wide limits.

The outstanding characteristic of these new agents is that they are capable of being almost perfectly retained or mordanted in the sheet, as formed on the wire of the paper-machine, after precipitation in the form of an insoluble salt, in any proportion, in the pulp by treatment with a suitable precipitant. For example, they may be added to pulp in an amount sufficient to produce a finished paper containing as high as 50% by weight of said insoluble salt. In contradistinction thereto, it is known, as has been stated 75 heretofore, that ordinary rosin size is retained with difficulty on the cellulose fibers in amounts over 8% (based on the weight of the finished product). This characteristic property of the new sizing agents renders possible 80 the retention in the sheet of larger proportions of inert materials (fillers) than are possible when rosin size is used.

It has been found, also, that these new sizing agents have, in many cases, as compared 85 with rosin size, enhanced waterproofing properties, and that they produce papers which have from three to six times the strength of rosin-sized papers prepared from the same pulp. Of importance is the fact 90 that they may be manufactured at a cost materially lower than that of rosin size.

The process of making these products consists generally in the liquid-phase oxidation of hydrocarbons or mixtures thereof, including both light and heavy petroleum distillates and waxes, the separation of organic oxygen-containing acids from the reaction mixture and the conversion of said acids to their corresponding water-soluble salts. 100

Although organic acid products may be derived from substantially all light and heavy distillates, I prefer to use as starting material a cheap petroleum distillate such as a 36° to 5 40° Baumé fuel oil distillate, obtainable from a crude petroleum having a paraffine base, and having a distillation range substantially as follows:

|                        |         |
|------------------------|---------|
| Initial boiling point  | 260° C. |
| 10 50% distilled up to | 321° C. |
| 15 75% distilled up to | 341° C. |
| 20 87% distilled up to | 360° C. |

The hydrocarbons present in this particular 15 distillate will belong almost exclusively to the saturated aliphatic, or paraffine, series, and in general correspond to substances containing on the average approximately twenty atoms of carbon to the molecule. When the fuel 20 oil distillate of the above type and character is subjected to rather thorough oxidation, it is converted practically entirely into a body heavier than water; insoluble in water and in the petroleum distillate; readily soluble in an 25 aqueous solution of a caustic alkali or an alkali metal carbonate to form a water-soluble soap. This soap may be decomposed and transformed into an insoluble metal salt of the acid by treatment with the suitable 30 organic salt of a metal; for example, aluminum sulfate or alum.

The invention will be described herein-after by reference to the accompanying dia- 35 grammatic drawing which illustrates one form of apparatus suitable for carrying out the oxidation process.

The oxidation step proper takes place in an upright cylindrical reaction vessel or oxidizer 1, which may be, for example, about 5 40 feet in diameter and about 16 to 18 feet in height. The oxidizer 1 may be made of any suitable material such as iron or steel and should be capable of withstanding pressures up to 350 pounds per square inch. Prefer- 45 ably, the oxidizer 1 should be made of or lined with material which is resistance to the corrosive action of the reaction mixture; for example, provided with an inner shell of aluminum or brick 2. The oxidizer is pro- 50 vided at a point near its lower end with a tight coil 3 which serves as a heating or cooling coil as required. Suitable means, not illustrated, such as a jacket surrounding the 55 oxidizer, also may be used to control the temperature of the oxidation reaction. At a point between the lower end of the oxidizer 1 and the tight coil 3 is an air spray pipe 4 connected by pipe line 5 to an air compressor 6. Air spray pipe 4 is so designed that air is ejected from it in the form of fine bubbles. 7, 8 and 9 are a valved hydrocarbon supply pipe, a valved liquid discharge pipe and a 60 valved gas discharge pipe, respectively. 10 65 is a pressure gauge, and 11 is a thermometer.

12 is a force pump for circulating oil from the separating tank 13 to the oxidizer 1.

The valved discharge pipe 8 extends through the top of the oxidizer 1 to a point a short distance below the top, thereby providing an air space or air cushion over the body of oil 14 therein.

15 is a jacketed condenser connected to the oxidizer 1 by means of the valved liquid discharge pipe 8. 22 is a valved pipe for conveying liquid from the bottom of the condenser 15 to the top of the settling tank 13, while 21 is a pipe connecting the top of condenser 15 with the bottom of the absorbing tower 16. 17 is an oil supply tank connected to the top of the settling tank 13 by the valved supply pipe 18. 19 and 20 are pressure gauges and 23 and 24 are valved exit lines for leading off gaseous and liquid products from the absorbing tower 16.

The process is carried out in the apparatus illustrated as follows:

A petroleum hydrocarbon oil, such as for example the hereinbefore described 36° to 40° Baumé fuel oil distillate, is charged into 90 oxidizer 1, a small amount of an oxidizing catalyst such as a compound of manganese, copper or iron, say manganese oleate, amounting to about 0.1 percent of the weight of the oil is added and the mixture heated up to a 95 temperature in the neighborhood of 120° C. or higher, preferably to about 135-140° C., and an oxidizing gas, preferably air, is supplied through the spray pipe 4. Gases are permitted to accumulate in the oxidizer 100 until the desired pressure is reached, after which the pressure is maintained or regulated by controlling the discharge of gases through the valved gas discharge pipe 9. The pressure may vary considerably, say from 250 to 320 pounds per square inch. The preferred 105 pressure will depend upon a number of conditions, including the temperature maintained, the kind of hydrocarbon mixture under treatment, the rate of air supply and, if oxygen-enriched air is used, upon the richness of the oxygen supply. It is preferred to carry out the oxidation process under such 110 conditions that the reaction is substantially self-sustaining. In general, the reaction is self-sustaining at a temperature of about 135°-140° C., and at a pressure of about 200-300 pounds per square inch, with the hydro carbon under treatment, although 115 temperatures and pressures may vary between wide limits. Thus, for example, oxidation has been observed at a temperature as low as 100° C.; it is more rapid above 120° C., and the temperature may be allowed to rise to 155° C. with satisfactory results under 120 some circumstances. Therefore, while I prefer to carry out the oxidation process at a temperature at which the reaction rate is fairly rapid, say 135°-140° C., it is to be 125 understood that the invention includes the 130

employment of all suitable temperatures at which oxidation takes place.

During the oxidizing treatment, as is stated above, gases collecting in the upper end of oxidizer 1 are released through the pipe 9. These gases contain practically no oxygen, but do contain carbon dioxide, nitrogen and varying quantities of volatile acids, ketones and other products of the oxidation. 5 The volatile acids, ketones and other products may be condensed in a suitable condenser 25 and further treated for the recovery of formic acid, mixed light ketones, etc.

The body of oil 14 being constantly augmented by oil drawn from the upper portion of the separating tank 13, overflows through pipe 8, into condenser 15 and thence into the separating tank through pipe 22. The overflow contains heavy organic carboxylic and hydroxy-carboxylic acids, partially oxidized hydrocarbons and unoxidized oil. The rate of flow through the oxidizer is so maintained that never more than 10%, and preferably not more than 4-5%, of the 20 heavy organic acids are present in the overflowing mixture. This would be at about the rate such that the whole amount of oil in the oxidizer is renewed once in 24 hours. Also, the volume of air passed through the oil naturally must be regulated to give the correct 25 degree of oxidation. Deficiencies in the volume of oil circulating through the apparatus may be made up by adding, either continuously or intermittently, fresh raw material 30 from an oil supply tank 17, through valved pipe line 18.

Uncondensed products pass out of condenser 15 into absorbing tower 16 which tower is partially filled with broken limestone, where a part of the uncondensed products may be absorbed. Unabsorbed gases 40 pass out of tower 16 through pipe line 24, and condensate may be drawn from the bottom of said tower through the valved pipe line 23.

The oxidation products present in the overflow from oxidizer 1, being heavier than the unoxidized oil and insoluble therein, settle to the bottom of the separating tank 13 50 and may be drawn therefrom through the valved pipe line 26, leading from the bottom of said tank, into a still 27. These oxidation products have been found to consist mainly of organic acids of relatively high 55 molecular weight,—comprising carboxylic and hydroxy-carboxylic acids—together with heavier ketones and other bodies.

The crude mixture of acidic oxidation products after having been separated from the unoxidized oil and only partly oxidized oil in the separating tank 13 and drawn into the still 27, is there purified by treatment with live steam. The temperature of the mixture may be brought up to about 150° C. 60 by suitable means such as a tight steam coil

or steam jacket (not shown). During this heating operation water and ketones are distilled off. Then steam is bubbled through the mixture until all volatile bodies have been removed. Upon cooling the contents 70 of the still, some heavy sludge may be separated out. This is carefully drawn off, and then the purified organic oxygen-containing acids, or "size acid", are withdrawn into a suitable vessel for neutralization (not shown). Preferably the said "size acid" is neutralized by agitation with the required amount of caustic soda solution or soda ash solution, forming water-soluble alkali metal soaps of the organic oxygen-containing acid. 80

The water-soluble alkali metal soap of the said "size acid" may be added to the pulp in the beating engine in much the same manner as ordinary rosin size. Upon addition of the requisite amount of a suitable precipitant, as, for example, alum or aluminum sulfate, it is caused to become fixed or mordanted on the cellulose fibers in almost any proportion. Preferably an excess of 85 aluminum salt is used.

The sizing agents made according to the above described process are rather dark in color, but the precipitated aluminum salts are comparatively light colored. The sizing agents may be bleached, if desired, according to the following procedure: An excess of the alkali solution is added to the purified "size acid" and chlorine gas passed therethrough until the desired color is obtained. This operation may be carried out 90 either with or without heating. Any excess alkalinity in the bleached sizing agent may be neutralized by the addition of the requisite amount of a suitable neutralizing agent (e. g., a mineral acid). 100

Another feature of this invention is that, by a suitable choice of petroleum distillates, there may be prepared, according to the process described, paper sizing agents which have different characteristics or properties. 105 Thus, for example, I have found that those sizing agents which have been prepared from distillates containing little or no crystalline bodies (wax) form the strongest papers, at some sacrifice in water-repelling properties, and that these sizing agents which have been prepared from distillates containing much wax and considerable quantities of unsaponifiable matter do not add materially to the strength of the paper but do offer relatively 110 very great water-repelling properties. I have found, further, that paraffine wax may be oxidized so that 10-20% of the mass is soluble in an aqueous solution of an alkali to form an emulsifiable product which may be incorporated in papers in the form of water-insoluble, unsaponifiable, bodies, in almost any proportions, for example in amounts up to 50% 115 of the final weight of the finished papers. 120

Although in the above description I have 125

disclosed a continuous process for the preparation of the organic oxygen-containing acid products, I have found that the operations may be carried out with equally good results by a batch process. While I have described the use of a catalytic agent (manganese oleate) in the oxidizing operation, it is to be understood that the process is operative without the use of a catalyst, or with catalysts other than manganese oleate.

This application is a continuation in part of my co-pending applications Serial No. 588,073, filed Sept. 13, 1922, and Serial No. 642,638, filed May 31, 1923.

15 What I claim is:

1. As a product, a material adapted for use as a paper sizing agent and consisting essentially of water-soluble alkali metal salts of normally liquid water-insoluble, petroleum-insoluble, relatively high molecular weight aliphatic carboxylic and hydroxy-carboxylic acids, said product being further characterized in that it is capable of being retained in a paper in an amount up to 50% by weight.

2. As a product, a material adapted for use as a paper sizing agent and consisting essentially of water-soluble alkali metal salts of the normally liquid water-insoluble, petroleum-insoluble, relatively high molecular weight aliphatic carboxylic and hydroxy-carboxylic acids produced by the protracted liquid-phase oxidation of petroleum hydrocarbon mixtures at elevated temperatures not in excess of about 155° C. and at a pressure greater than atmospheric in the presence of an exciter of oxidation, said product being further characterized in that it is capable of being retained in a paper in an amount up to 50% by weight.

3. A sized paper comprising a fibrous cellulosic web and a sizing material, said sized paper being characterized in that it has a greater water-repelling capacity and a greater strength than that possessed by a rosin-sized paper containing the same amount of sizing material and further characterized in that its sizing material consists essentially of water-insoluble metal salts of water-insoluble petroleum-insoluble, relatively high molecular weight aliphatic carboxylic and hydroxy-carboxylic acids.

4. A sized paper comprising a fibrous cellulosic web and a sizing material, said sized paper being characterized in that it has a greater water-repelling capacity and a greater strength than that possessed by a rosin-sized paper containing the same amount of sizing material and further characterized in that its sizing material consists essentially of water-insoluble metal salts of the water-insoluble, petroleum-insoluble, relatively high molecular weight aliphatic carboxylic and hydroxy-carboxylic acids produced by the protracted liquid-phase oxidation of petroleum hydro-

carbon mixtures at elevated temperatures not in excess of about 155° C. and at a pressure greater than atmospheric in the presence of an exciter of oxidation.

In testimony whereof, I affix my signature.

ARTHUR W. BURWELL.

70

75

80

85

90

95

100

105

110

115

120

125

130